

Feb. 28, 1956

H. WALKER ET AL

2,736,080

MANUFACTURE OF THIN SHEETS OR PLATES OF HEAT-TREATED  
MATERIAL SUITABLE FOR THE DIELECTRICS OF  
CAPACITORS AND FOR OTHER PURPOSES

Filed Feb. 28, 1951

2 Sheets-Sheet 1

FIG. 1.



FIG. 2.



Inventors

Herbert Walker and  
Tz'u En Shen

By

Webb, Mackay & Burden

Attorneys

Feb. 28, 1956

H. WALKER ET AL  
MANUFACTURE OF THIN SHEETS OR PLATES OF HEAT-TREATED  
MATERIAL SUITABLE FOR THE DIELECTRICS OF  
CAPACITORS AND FOR OTHER PURPOSES

2,736,080

Filed Feb. 28, 1951

2 Sheets-Sheet 2

FIG. 3.



Inventors

Herbert Walker  
Teu En Shen

By

Cobb Mackay + Burden  
Attorney

# United States Patent Office

2,736,080

Patented Feb. 28, 1956

1

2,736,080

## MANUFACTURE OF THIN SHEETS OR PLATES OF HEAT-TREATED MATERIAL SUITABLE FOR THE DIELECTRICS OF CAPACITORS AND FOR OTHER PURPOSES

Herbert Walker and Tzu En Shen, London, England, assignors to British Dielectric Research Limited, London, England, a British company

Application February 28, 1951, Serial No. 213,107

Claims priority, application Great Britain March 9, 1950

6 Claims. (Cl. 25—156)

In the manufacture of sheets or plates of material suitable for the dielectrics of capacitors the attainment of small thickness is obviously important. It is also difficult of attainment with materials which in the early stages of manufacture are in the form of powder given cohesion by appropriate means. Such materials are not readily made to flow into thin layers by moulding, pressing, or rolling unless excessive quantities of other materials are added. These additions have disadvantageous results, either in later stages of manufacture or in the final product. Such materials if they can be formed into thin plates are usually very fragile and difficult to handle in later stages of the manufacture. Materials to which these comments apply are ceramic bodies, such as titanium dioxide (rutile) and titanates of barium and strontium and of other elements. The present invention provides a new method of manufacturing thin sheets or plates from such materials in which the limitations indicated above are not present.

The term thin as used herein means of a thickness comparable with that of cellulose paper.

By cellulose paper is meant paper made from cellulose pulp, such as wood pulp or pulp made from cotton or linen rag or natural fibres, such as cotton or manilla, or mixtures of any of these materials.

The first stage of the manufacture is to produce a cellulose paper loaded with the powder to a high degree, for instance to 90% or 95% by weight, and having an appropriate thickness, for instance 5 mils (.13 mm.). This stage is preferably finished by rolling or pressing so as to obtain as dense a paper as possible. In the next stage the paper is heated so as to burn off the other ingredients of the paper and is continued until the powder is brought to the temperature at which it sinters to form a sheet of strongly coherent material.

This sheet is of substantially uniform thickness. The limit of thinness is determined mainly by the capacity to produce sufficiently thin paper. The material in the final form is generally rigid so that any shaping required is preferably done while the material is still in the form of paper. In many cases flat sheets will be required.

It will be seen that the method imposes certain limitations on the choice of materials to which it can be applied, particularly as to their properties over a large range of temperature. They should be stable and unaffected by heat at the temperature at which the other ingredients of the paper are driven off and should then be capable of being softened and sintered at a substantially higher temperature. Suitable materials are, for instance, ceramic materials and glass. Small quantities of flux may be added to assist sintering.

The remainder of the paper is preferably substantially wholly cellulose fibres and small quantities of binders which are commonly employed in the paper industry such as starch, dextrose or gelatine. The paper may be made in known manner, preferably beating

2

the cellulose fibres to the high degree appropriate for the making of very thin paper, such as condenser tissue. In the later stages the powdered substance is added and beaten thoroughly with the cellulose fibres. The web of paper is then taken up in the usual way, dried and preferably calendered.

As already indicated the heating takes place in two stages at substantially different temperatures. In the first the conditions are oxidising so that combustion of the cellulose can take place. In the latter stage the conditions are determined by the nature of the material and the properties which it is desired that the finished product shall have.

In order to give the finished plates or sheets the desired form, it may be necessary or advantageous to hold the paper between shaping surfaces during the heat treatment. The attainment of a flat sheet can be assisted by ensuring uniformity of the thickness and structure of the paper and of the heat treatment as far as possible. It may be further ensured by placing the paper between flat plates for the heat treatment.

The following are examples of methods of manufacture in accordance with the invention. These examples describe the manufacture of sheet materials of high dielectric constant suitable for use as capacitor dielectrics.

### Example I

The first stage is the preparation of a paper loaded with barium titanate. This is carried out by mixing together a cellulose pulp, such as is used in paper making, with barium titanate and a small quantity of bentonite. The ingredients are used in the following proportions by weight:

|    |                                |    |
|----|--------------------------------|----|
| 35 | Cellulose pulp (solid content) | 1  |
|    | Bentonite                      | 1  |
|    | Barium titanate                | 98 |

The slurry so obtained is spread into sheets, dried and rolled by a normal paper making process to produce thin sheets resembling paper. The final pressure applied may be of the order of 10 tons per square inch.

The sheets thus obtained are arranged between flat zircon plates and fired. Four sheets for example may be stacked between one pair of zircon plates. The best firing temperature is 1305° C. although this may be varied from 1280°—1330° C.

The total firing time is three hours including a period of  $\frac{1}{2}$  hour during which the cellulose is burnt out, the temperature rising from 20° C. to 500° C., a further period of  $\frac{1}{2}$  hour during which the temperature rises to and is held at the sintering temperature and a period of 2 hours for cooling.

The proportion of ingredients given above can be varied between the following limits:

|                 | Percent          |
|-----------------|------------------|
| Cellulose       | $\frac{1}{2}$ —2 |
| Bentonite       | $\frac{1}{2}$ —1 |
| Barium titanate | 99.97            |

In all cases a strongly coherent sheet having a dielectric constant between 1,000 and 2,000 at room temperature is obtained. If higher proportions of cellulose are used the sheet obtained is liable to be too porous for use as a capacitor dielectric. If less than  $\frac{1}{2}\%$  of cellulose is used the loaded paper is too weak to handle. It is preferred to use 1% of cellulose.

For making small quantities of the sheet material described in the example, it is possible to obtain the cellulose pulp by breaking down paper. For example, a suitable pulp can be obtained by milling 1 gm. of capacitor tissue with 100 cc. of distilled water for four hours in a plane-

tary ball mill. To mix in the barium titanate, 98 grams of the powder and 1 gram of bentonite are added to the pulp together with another 100 cc. of water and the milling is continued for another four hours.

Small quantities of the loaded paper can be prepared by drying the pulp on filter paper under suction followed by heating in an oven at 80-90° C. The filter paper can be removed from the loaded paper before or after the oven drying.

*Example II*

In this example the ingredients used, in proportions by weight are:

|                                |    |
|--------------------------------|----|
| Cellulose pulp (solid content) | 1  |
| Bentonite                      | 1  |
| Titanium dioxide               | 98 |

the same process as described in Example I is used but the firing temperature is 1450° C. The firing times are the same.

*Example III*

In this example the ingredients used, in proportions by weight are:

|                                |    |
|--------------------------------|----|
| Cellulose pulp (solid content) | 1  |
| Bentonite                      | 1  |
| Magnesium titanate             | 98 |

the same process as described in Example I is used but the firing temperature is 1400° C. The firing times are the same.

Although the method of manufacture has been referred to particularly in connection with the preparation of dielectric bodies for capacitors, it is to be understood that it may also be used for the preparation of materials for other purposes. The applicability of the method in such cases will be recognised by a consideration of the nature of the materials to be used and the form of the final product required. It is only necessary that the material will withstand the heat necessary to destroy the cellulose and will itself sinter to form a thin plate. The method is applicable to the manufacture of thin sheets or plates from powdered glass alone or mixed with dielectric ceramic materials (particularly ceramic materials with high dielectric constants), powdered metals, for example tantalum, aluminium and titanium, silicon carbide and mixtures of carbon, silica and/or silicates. The mixtures of carbon, silica and/or silicates are useful in the manufacture of electrical resistors. In such mixtures the carbon itself does not sinter but becomes incorporated in the ceramic material produced by the sintering of the silicon and/or silicates present. Silicon carbide is used when resistors in which resistance varies with voltage or current are required. When materials are used which are liable to oxidise at the sintering temperature precautions are taken to exclude oxygen during the latter part of the heat treatment.

While the upper limits of the thickness of the sheets or plates which can be made by the method of the invention from a single sheet of loaded paper is controlled only by the thickness of the loaded paper sheet there would be little advantage in using the method for the manufacture of sheets or plates thicker than about 10 mils (.25 mm.) since such plates or sheets would probably be more easily made by known dry pressing processes.

In the accompanying drawing Figures 1 and 2 show two alternative forms of capacitor manufactured in accordance with the invention and Figure 3 shows a process in accordance with the invention.

The capacitor shown in Figure 1 is a stack type made up of a number of plates 1 of a material of the kind described in the examples. Each plate is formed on both sides with metallised layers in accordance with normal practice, the layer 2 on the upper surface extending over one end of the plate and onto the lower side and the layer 3 on the lower side extending over the other end and onto

the upper side, as shown. Metal connecting wires 4 and 5 are soldered to the ends of the stack.

Figure 2 shows a single plate capacitor consisting of a circular plate 6 of a material manufactured in accordance with one of the examples provided with metallised layers on its upper and lower surfaces. The layer 7 on the upper surface has soldered to it a connecting wire 8. A similar wire 9 is soldered to the lower metallised layer.

Referring to Figure 3 of the drawings an aqueous dispersion 10 of cellulose fibres and a powdered material, formed by a beating process, is contained in a vessel through which a continuous gauze 11, of the kind used in paper making, passes round a roller 12 in a clockwise direction. The gauze passes from the dispersion beneath the heater 13 and over a tray 14 which is evacuated by a pump 15.

As the gauze rises from the surface of the dispersion 10, it picks up a layer 16 which is carried over the tray 14 and beneath the heater 13 and is dried sufficiently to 20 make it into a self-supporting sheet. The sheet 17 is lifted continuously from the gauze 11 and passes between at least one pair of calender rolls 18, 19. During 25 passage through these rolls it is compressed to the required thickness and density. From the rolls the sheet passes on to a conveyor 20 which carries it through a cutting machine 21 where it is reduced to the required shapes for example discs.

In the drawing, discs 22 are shown issuing from the machine 21. These are placed by hand into ceramic dishes 23 which are fed successively into a firing kiln 24. In the kiln the discs are fired in the manner described in the examples. If desired, the discs, before firing, can be arranged between flat zircon plates which are not affected by the temperatures reached in the firing kiln.

Both forms of capacitor are provided with a protective layer of insulating wax or varnish.

What we claim as our invention is:

1. A method of manufacturing a thin, strongly coherent electrically insulating sheet from a ceramic powder which comprises preparing a suspension of cellulose fibers and said powder in an aqueous liquid by a beating process, taking up a layer of said suspension of not more than about 10 mils thickness on a pervious support, the relative proportions of cellulose and ceramic powder in said suspension being such that at least 95% by weight of the solid content of said layer consists of said powder, draining liquid contained in said layer through said support, drying said layer until it is self supporting, removing said layer as a sheet from said support, consolidating said sheet by the application of pressure and heating said sheet under oxidising conditions first to burn off the cellulose and then at a higher temperature to sinter said powder and form a sheet of strongly coherent material.

2. A method of manufacturing a thin, strongly coherent electrically insulating sheet from a ceramic powder, selected from the group consisting of titanium dioxide and metallic titanate powders with or without small quantities of additives, which comprises preparing a suspension of cellulose fibers and said powder in an aqueous liquid by a beating process, taking up a thin layer of said suspension of not more than about 10 mils thickness on a pervious support, the relative proportions of cellulose and ceramic powder in said suspension being such that at least 95% by weight of the solid content of said layer consists of said powder, draining liquid contained in said layer through said support, drying said layer until it is self supporting, removing said layer as a sheet from said support, consolidating said sheet by the application of pressure and heating said sheet under oxidising conditions first to burn off the cellulose and then at a higher temperature to sinter said powder and form a sheet of strongly coherent material.

3. A method of manufacturing a thin, strongly coherent electrically insulating sheet from a ceramic powder, selected from the group consisting of titanium dioxide

and metallic titanate powders with or without small quantities of additives which comprises preparing a suspension of cellulose fibers, bentonite and said powder in an aqueous liquid by a beating process, taking up a layer of said suspension of not more than about 10 mils thickness on a pervious support, the relative proportions of said ingredients of said suspension being such that the solid content by weight of said layer is cellulose ½-2%, bentonite ½-1% and ceramic powder 99-97%, draining liquid contained in said layer through said support, drying said layer until it is self supporting, removing said layer as a sheet from said support, consolidating said sheet by the application of pressure and heating said sheet under oxidising conditions first to burn off the cellulose and then at a higher temperature to sinter said powder and form a sheet of strongly coherent material.

4. A method of manufacturing a thin, strongly coherent electrically insulating sheet from a ceramic powder, which comprises preparing a suspension of cellulose fibers and said powder in an aqueous liquid by a beating process, taking up a layer of said suspension of not more than about 10 mils thickness on a pervious support, the relative proportions of cellulose and ceramic powder in said suspension being such that at least 95% by weight of the solid content of said layer consists of said powder, draining liquid contained in said layer through said support, drying said layer until it is self supporting, removing said layer as a sheet from said support, stacking a plurality of said sheets, consolidating said stacked sheets by the application of pressure and heating under oxidising conditions first to burn off the cellulose and then at a higher temperature to sinter said powder and form a sheet of strongly coherent material.

5. A method of manufacturing a thin, strongly coherent electrically insulating sheet made from a ceramic powder, selected from the group consisting of titanium dioxide and metallic titanate powders with or without small quantities of additives, which comprises preparing a suspension of cellulose fibers and said powder in an aqueous liquid by a beating process, taking up a layer of said suspension of not more than 10 mils thickness on a pervious support, the relative proportions of cellulose and ceramic powder in said suspension being such that at least 95% by weight of the solid content of said layer consists of said powder, draining liquid contained in said layer through said support, drying said layer until it is self supporting, removing said layer as a sheet from said support,

stacking a plurality of said sheets, consolidating said stacked sheets by the application of pressure and heating under oxidising conditions first to burn off the cellulose and then at a higher temperature to sinter said powder and form a sheet of strongly coherent material.

- 5 6. A method of manufacturing a thin, strongly coherent electrically insulating sheet from a ceramic powder, selected from the group consisting of titanium dioxide and metallic titanate powders with or without small quantities of additives which comprises preparing a suspension of cellulose fibers, bentonite and said powder in an aqueous liquid by a beating process, taking up a layer of said suspension of not more than about 10 mils thickness on a pervious support, the relative proportions of said ingredients of said suspension being such that the solid content of weight of said layer is cellulose ½-2%, bentonite ½-1% and ceramic powder 99-97%, draining liquid contained in said layer through said support, drying said layer until it is self supporting, removing said layer as a sheet from said support, stacking a plurality of said sheets, consolidating said stacked sheets by the application of pressure and heating under oxidising conditions first to burn off the cellulose and then at a higher temperature to sinter said powder and form a sheet of strongly coherent material.
- 10 15 20 25

#### References Cited in the file of this patent

#### UNITED STATES PATENTS

|    |           |                      |                |
|----|-----------|----------------------|----------------|
| 30 | 1,152,060 | Sturm et al. -----   | Aug. 31, 1915  |
|    | 1,447,347 | Kirschbraum -----    | Mar. 6, 1923   |
|    | 2,063,102 | Jones -----          | Dec. 8, 1936   |
|    | 2,145,151 | Braunstein -----     | Jan. 24, 1939  |
|    | 2,330,106 | Bernstein -----      | Sept. 21, 1943 |
|    | 2,391,376 | Monack -----         | Dec. 18, 1945  |
|    | 2,486,410 | Howatt -----         | Nov. 1, 1949   |
|    | 2,499,229 | Rankine -----        | Feb. 28, 1950  |
|    | 2,539,446 | Lies -----           | Jan. 30, 1951  |
|    | 2,616,813 | Klasens -----        | Nov. 4, 1952   |
| 40 | 2,643,192 | Jonkers et al. ----- | June 23, 1953  |

#### FOREIGN PATENTS

|         |                     |               |
|---------|---------------------|---------------|
| 574,577 | Great Britain ----- | Jan. 11, 1946 |
|---------|---------------------|---------------|

#### OTHER REFERENCES

45 The Bible, Exodus, ch. 5, verses 6-8, (King James Version); Collins Clear Type Press, London, Eng. (1949).